

# United States Patent Office

2,781,262

Patented Feb. 12, 1957

1

2,781,262

## ALUMINUM-BASE ALLOY

Harold Ernest Gresham, Little Eaton, Alec George Farnsworth, Derby, Douglas W. Hall, Tynemouth, and William Michael Doyle, Slough, England, assignors to Rolls-Royce Limited, Derby, England, a corporation of Great Britain

No Drawing. Application October 21, 1953,  
Serial No. 387,524

Claims priority, application Great Britain  
October 25, 1952

5 Claims. (Cl. 75—143)

This invention relates to an improvement in aluminum-base alloys.

Among the objects of the present invention are to improve the creep and tensile properties of the aluminum-base alloys disclosed in British Patents Nos. 686,819 and 686,820, published January 28, 1953. These British patents disclose two alloys closely resembling one another in composition analysis, one of them (686,819) primarily intended to be used in the forged state after direct chill casting, and the other (686,820) primarily intended to be used in the cast condition.

The aluminum-base alloy which is shown in said British patents, and which is improved in certain properties by the invention hereinafter described, has the following typical approximate composition analysis:

Element:

|                     |                                       |
|---------------------|---------------------------------------|
| Copper              | About 5%.                             |
| Nickel              | About 1%.                             |
| Silicon             | About 0.15%.                          |
| Titanium            | About 0.2%.                           |
| Manganese           | About 0.25%.                          |
| Iron                | About 0.25%.                          |
| Antimony (optional) | About 0.25%.                          |
| Cobalt              | About 0.25%.                          |
| Balance             | Essentially aluminum plus impurities. |

The permissible ranges for the several constituents, other than residual aluminum, are set forth in detail in the British patents to which reference is hereby made. The following summarizes a portion of the disclosure contained in said patents.

**Copper.**—Below 4% copper the creep strength at high temperature (for example, at 300° C.) begins to fall off although it remains good down to about 3.5%. Above 6% copper there is a liability to segregation when the alloy is used in ordinary sand casting but, if the alloy is to be direct chill cast with a view to subsequent forging, the copper is preferably around 6% and can be tolerated up to 7% without serious segregation.

**Nickel.**—Below 0.5% nickel the alloy loses creep strength at elevated temperature. Above 1.5% it tends to become brittle, though if brittleness is comparatively unimportant nickel may be present up to about 2%.

**Silicon.**—Silicon is a normal impurity to be kept low. In general it is preferred that the silicon should be less than 0.25% and preferably in the approximate range 0.10% to 0.20%. When silicon is above 0.45% the creep strength of the alloy is seriously affected.

**Titanium.**—Titanium is essential for creep strength and as a refiner when used in quantities ranging from about 0.10% to about 0.25%, the preferred amounts being about 0.2%. When more than 0.30% of titanium is present there is a tendency to segregation on casting.

**Iron.**—Iron is a normal impurity to be kept low. Using commercially obtainable materials iron cannot be

2

expected to be much below about 0.10%, and in normal foundry practice it can be held to within the approximate range 0.20% to 0.30%. Iron can be tolerated up to 1%, but above that amount there is a tendency to embrittlement and loss of ductility.

**Manganese.**—Manganese is likewise essential for creep strength. When more than 0.6% is present there is a tendency to embrittlement and segregation.

**Antimony.**—When the alloy is intended to be used for a casting, antimony should desirably be present in combination with cobalt, mentioned below, in order to achieve good castability and creep strength. Not more than about 0.50% should be present in any event. The preferred amount is less than 0.30%.

**Cobalt.**—This element is essential for creep strength and good castability. If used without antimony, as for example in an alloy to be forged after direct chill casting, the cobalt should not exceed about 0.50%. If antimony and cobalt are both present, as in an alloy intended to be used for a casting, a total of antimony and cobalt together exceeding about 0.60% would produce a tendency to segregation, embrittlement.

Reference is made in the above-mentioned British patents to certain other elements which, if present in small quantities, can be tolerated or may optionally be included for improved qualities of castability or creep strength. One of these is zirconium which, said patents state, may be added up to about 0.4%, provided the total content of zirconium plus titanium does not exceed 0.5%.

According to the present invention a small quantity of cadmium, preferably about 0.10%, is added to the above-described alloy of the British patents, either to the form thereof which omits zirconium, or the form thereof which includes zirconium.

The substantial advantages from the addition of the cadmium begin to appear when about 0.05% thereof has been added. If the percentage of cadmium exceeds about 0.20% in an alloy intended for forging, the forging material becomes hot-short, that is, tends to become brittle under the forging hammer and to develop cracks. However, where the alloy is to be cast and not forged, cadmium may be added in amounts up to as much as 0.50%.

The addition of cadmium effects a major increase in the ultimate tensile strength at room temperature of the aluminum-base alloy above referred to, and also a substantial increase in creep strength at temperatures on the order of 200° C. These beneficial effects are achieved without substantially lessening the ultimate tensile strength or the creep strength of the material at higher temperatures such as 300° C.

### Example 1

Two alloys were made up and on analysis found to have the respective composition analyses set forth below. Of these, alloy A1 is very similar to the alloys disclosed in British Patent 686,820 and is of the type intended for ordinary casting. Alloy B1 is an example of an alloy according to this invention including cadmium.

|              |  | Alloy A1 | Alloy B1 |
|--------------|--|----------|----------|
| Copper       |  | 4.93     | 4.96     |
| Nickel       |  | 1.02     | 0.99     |
| Silicon      |  | 0.12     | 0.12     |
| Titanium     |  | 0.24     | 0.21     |
| 65 Manganese |  | 0.26     | 0.26     |
| Iron         |  | 0.31     | 0.29     |
| Antimony     |  | 0.23     | 0.24     |
| Cobalt       |  | 0.25     | 0.25     |
| Cadmium      |  | 0        | 0.09     |
| Aluminum     |  | Balance  | Balance  |

The following tests were carried out on horizontally-cast material which had been solution treated for 24

## 3

hours at 530° C., quenched in boiling water and aged for 16 hours at 215° C.

At room temperature, specimens of the above were subjected to the 0.1% proof stress test, i. e., the stress in tons per sq. in. required to produce 0.1% permanent deformation. For alloy A<sub>1</sub> the stress was 10.4, for alloy B<sub>1</sub> it was 17.6, a difference of 69%.

At room temperature, the ultimate tensile strength, in tons per sq. in., of alloy A<sub>1</sub> was 17.2, and of alloy B<sub>1</sub> was 20.1, a difference of 16%.

At 300° C., the 0.1% proof stress in tons per sq. in., after soaking for 1 hour at 300° C., was 5.7 for alloy A<sub>1</sub> and 6.8 for alloy B<sub>1</sub>, a difference of 19%.

## Example 2

An alloy was made up similar to alloy B<sub>1</sub> above but containing zirconium, and was found to have the composition analysis set forth below under the heading alloy C<sub>1</sub>, which is an example of an alloy made according to this invention.

|           | Alloy C <sub>1</sub> |  |
|-----------|----------------------|--|
| Copper    | 4.94                 |  |
| Nickel    | 1.03                 |  |
| Silicon   | 0.10                 |  |
| Titanium  | 0.24                 |  |
| Manganese | 0.23                 |  |
| Iron      | 0.23                 |  |
| Antimony  | 0.26                 |  |
| Cobalt    | 0.24                 |  |
| Cadmium   | 0.09                 |  |
| Zirconium | 1.09                 |  |
| Aluminium | Balance              |  |

At room temperature the 0.1% proof stress in tons per sq. in., for alloy A<sub>1</sub> was 10.4 and for alloy C<sub>1</sub> was 16.3, a difference of about 56%, and the ultimate tensile strength in tons per sq. in. for alloy A<sub>1</sub> was 17.2 and for alloy C<sub>1</sub> was 19.4, a difference of about 12%.

At 300° C. the 0.1% proof stress, in tons per sq. in., after soaking at 300° C. for one hour, was 5.7 for alloy A<sub>1</sub> and 6.7 for alloy C<sub>1</sub>, a difference of about 17%, and after soaking for 400 hours was 5.25 for alloy A<sub>1</sub> and 6.45 for alloy C<sub>1</sub>, a difference of about 22%.

At 300° C. the ultimate tensile strength, in tons per sq. in., after soaking at 300° C. for one hour was 8.1 for alloy A<sub>1</sub> and 8.4 for alloy C<sub>1</sub>, a difference of about 3.5%; and after soaking at 300° C. for 400 hours was 8.15 for alloy A<sub>1</sub> and 9.1 for alloy C<sub>1</sub>, a difference of about 11%.

## Example 3

Two alloys were made up and heat treated as in Example 1. The composition analyses showed the following:

|           | Alloy A <sub>2</sub> | Alloy B <sub>2</sub> |
|-----------|----------------------|----------------------|
| Copper    | 4.97                 | 4.95                 |
| Nickel    | 1.06                 | 0.99                 |
| Silicon   | 0.12                 | 0.12                 |
| Titanium  | 0.17                 | 0.17                 |
| Manganese | 0.26                 | 0.26                 |
| Iron      | 0.24                 | 0.23                 |
| Antimony  | 0.23                 | 0.23                 |
| Cobalt    | 0.25                 | 0.25                 |
| Cadmium   | 0                    | 0.10                 |
| Aluminium | Balance              | Balance              |

In order to ascertain the effect of the addition of cadmium on creep strength at 200° C., specimens of the above alloys were tested to determine the stress required to produce 0.1% creep in 300 hours at 200° C., expressed in tons per sq. in. These tests indicated that the stress for alloy A<sub>2</sub> was 4.5, and for alloy B<sub>2</sub> was 6.4, a difference of about 42%.

## Example 4

Specimens were prepared in accordance with ordinary foundry practice of alloy pieces whose composition

## 4

analysis was found to be as shown in the table below. Alloy A<sub>3</sub> is a typical alloy in accordance with British Patent No. 686,819, primarily intended for forging. It differs from alloy A<sub>1</sub> and alloy A<sub>2</sub> of the previous examples chiefly in having a larger quantity of copper. Alloy B<sub>3</sub> is another example of an alloy made according to this invention.

|           | Alloy A <sub>3</sub> | Alloy B <sub>3</sub> |
|-----------|----------------------|----------------------|
| Copper    | 6.17                 | 6.12                 |
| Nickel    | 1.01                 | 1.08                 |
| Silicon   | 0.13                 | 0.13                 |
| Titanium  | 0.17                 | 0.17                 |
| Manganese | 0.26                 | 0.26                 |
| Iron      | 0.23                 | 0.21                 |
| Antimony  | 0.25                 | 0.26                 |
| Cobalt    | 0.26                 | 0.26                 |
| Cadmium   | 0                    | 0.10                 |
| Aluminium | Balance              | Balance              |

The following tests were carried out on material which had been solution treated for 24 hours at 540° C., quenched in water at 70° C., and aged for 16 hours at 215° C.

At room temperature, forged pieces of the above alloys gave the following results: The 0.1% proof stress, in tons per sq. in., for alloy A<sub>3</sub> was 14.2 and for alloy B<sub>3</sub> was 19.3, a difference of over 35%. At room temperature the ultimate tensile strength, in tons per sq. in., of alloy A<sub>3</sub> was 22.6 and of alloy B<sub>3</sub> was 25.5, a difference of about 12%.

At 300° C. the 0.1% proof stress in tons per sq. in., after soaking for one hour at 300° C. was 6.8 for alloy A<sub>3</sub> and 7.65 for alloy B<sub>3</sub>, a difference of about 12%.

## Example 5

A further example of this invention was prepared in accordance with ordinary foundry practice and was found to have the composition analysis shown below for alloy C<sub>3</sub>, which contains both cadmium and zirconium.

|           | Alloy C <sub>3</sub> |
|-----------|----------------------|
| Copper    | 5.89                 |
| Nickel    | 1.06                 |
| Silicon   | 0.17                 |
| Titanium  | 0.22                 |
| Manganese | 0.26                 |
| Iron      | 0.24                 |
| Antimony  | 0.25                 |
| Cobalt    | 0.27                 |
| Cadmium   | 0.10                 |
| Zirconium | 0.19                 |
| Aluminium | Balance              |

The following tests were carried out on material heat treated as mentioned under "Example 4."

At room temperature, forged pieces of the above alloy showed a 0.1% proof stress, in tons per sq. in., of 18.1, which is about 27% better than the same figure for alloy A<sub>3</sub>; and an ultimate tensile strength, in tons per sq. in., of 24.7, which is about 9% better than the same figure for alloy A<sub>3</sub>.

At 300° C., the 0.1% proof stress, after soaking at this temperature for 400 hours, was 6.45 for alloy A<sub>3</sub> and 6.90 for alloy C<sub>3</sub>, a difference of about 5%. At 300° C. the stress to fracture in 100 hours, in tons per sq. in., was approximately 5.2 for alloy A<sub>3</sub> and approximately 5.8 for alloy C<sub>3</sub>, a difference of about 11%.

Reference herein to "tons" means long tons of 2240 lbs. each. It is not claimed that the condition of cadmium alone produces any important improvement in creep properties at 300° C., although such addition does so at 200° C. as pointed out above. However, the addition of cadmium and zirconium together, as described, produces the above mentioned improvements at 200° C. and in addition brings about significant enhancement in these properties at 300° C.

What is claimed is:

1. An aluminum-base alloy of the class which consists by weight of about 5% copper, about 1% nickel, about 0.15% silicon, about 0.2% titanium, about 0.25% manganese, about 0.25% iron, up to about 0.25% antimony, about 0.25% cobalt and the balance essentially aluminium plus impurities, characterized in that the alloy contains by weight about 0.05% to 0.50% of cadmium.

2. An aluminum-base alloy of the class which consists by weight of about 5% copper, about 1% nickel, about 0.15% silicon, about 0.2% titanium, about 0.25% manganese, about 0.25% iron, up to about 0.25% antimony, about 0.25% cobalt and the balance essentially aluminium plus impurities, characterized in that the alloy also contains by weight about 0.05% to 0.5% of cadmium and up to about 0.4% of zirconium.

3. An aluminum-base alloy of the class which consists by weight of about 5% copper, about 1% nickel, about 0.15% silicon, about 0.2% titanium, about 0.25% manganese, about 0.25% iron, up to about 0.25% antimony, about 0.25% cobalt and the balance essentially aluminium plus impurities, characterized in that the alloy also contains by weight about 0.05% to 0.5% of cadmium and about 0.19% of zirconium.

4. An aluminium-base alloy of the class which consists by weight of about 5% copper, about 1% nickel, about 0.15% silicon, about 0.2% titanium, about 0.25% manganese, about 0.25% iron, up to about 0.25% antimony, about 0.25% cobalt and the balance essentially aluminium plus impurities, characterized in that the alloy also contains by weight about 0.10% of cadmium.

5. An aluminum-base alloy of the class which consists by weight of about 5% copper, about 1% nickel, about 0.15% silicon, about 0.2% titanium, about 0.25% manganese, about 0.25% iron, up to about 0.25% antimony, about 0.25% cobalt and the balance essentially aluminium plus impurities, characterized in that the alloy also contains by weight about 0.10% of cadmium and about 0.19% zirconium.

References Cited in the file of this patent

UNITED STATES PATENTS

20 2,063,942 Nock ----- Dec. 15, 1936

FOREIGN PATENTS

686,819 Great Britain ----- Jan. 28, 1953  
686,820 Great Britain ----- Jan. 28, 1953